

## UNITED STATES PATENT OFFICE

EUGENIUSZ BAZYLEWICZ-KNIAZYKOWSKI AND KAZIMIERZ PARTYKA, OF SOCHACZEW,  
POLAND

## METHOD OF PRODUCING SMOKELESS GUNPOWDER

No Drawing. Application filed June 25, 1930, Serial No. 463,816, and in Poland February 24, 1927.

This application is a continuation in part of our application Serial No. 233,309, filed November 14, 1927.

This invention provides the possibility of 5 producing good smokeless gunpowder for sporting and practice purposes without using special machines, but only the machines ordinarily used in the manufacture of carbine gunpowder, by the suitable preparation of 10 the gunpowder mass and the introduction of additional operations directly after having pressed the gunpowder threads.

As is generally known carbine gunpowder, in order to burn progressively, must be made 15 from gelatinized nitrocellulose and the surface of the gunpowder grains must be subjected to an additional treatment for slower combustion in the chamber. Entirely different properties are required of sporting 20 and practice gunpowders. The combustion of these gunpowders must be very rapid, so that even at small pressures in the chamber (400-500 atmospheres in the case of sporting guns) there will be complete combustion 25 when a shot is being fired.

The method according to the present invention provides the possibility, while using only the machines ordinarily used for the manufacture of carbine gunpowder, (other 30 machines may also be used), of obtaining very uniform sporting and practice gunpowders in the form of exceedingly thin-walled tubular threads, having an ideal combustion and any desired ballistic properties, which 35 latter can be easily regulated during the process of production.

The walls of the tubular threads of powder prepared by our method have a thickness of 0.03-0.1 mm., and powder tubes of 40 such thin walls could not be obtained by the pressure usually employed hitherto with a pitch or thorn matrix, as every matrix would unavoidably be immediately blocked with portions of the powder material.

The method according to the present invention is as follows. Explosive material is 45 gelatinized by means of suitable solvents, such as, for instance, alcohol and ether, as in the case of progressive powders. It is 50 then extruded in the form of continuous

cylindrical threads having a diameter of 0.3-1.5 mm. according to the kind of powder, e. g. 0.8 mm., the thread formed containing solvent to an amount which varies between 130-150% of the weight of the dry mass. The thread is then partly dried in order to make it slightly stable; it may be dried, for example, to such an extent that it contains a weight of water which is not less than the weight of the original dry mass. 55 The drying may, for example, be carried out by subjecting the thread to 50° C. for 1-2 minutes (or until the solvent content is 95-100% of the weight of the dry mass), 60 preferably in a fluid, which may be the air. 65 The thread thus obtains a dried, somewhat hard, surface whilst the core-portion remains perfectly soft, and it is then plunged into a fluid having a temperature (e. g. of 45-80° C. according to the nature of the powder) 70 somewhat higher than the boiling point of the solvents used or of one of the ingredients of extruded material. The fluid is chosen such that it does not act chemically upon the powder. The temperature of the fluid bath 75 evaporates the solvent contained in the thread and creates pressure from the centre of the thread towards the periphery, which latter, however, is relatively hard, and consequently a channel is blown throughout the 80 length of the thread. Immersion in the bath lasts about 10 to 25 minutes and the partly dried threads are cut in the usual way, preferably while still moist so as to eliminate 85 danger of explosion. The cut grains are then dried, soaked, polished, graphited or coated with camphor, centralite or other coating materials.

The explosive material being gelatinized 90 may contain 0.1-0.5% of graphite for the purpose of increasing the electrical conductivity. It may also contain 6-10% of water for the purpose of obviating the brittleness of the threads when formed. The stability of the material, also, may be increased by 95 adding diphenylamine, urea derivatives, etc. to the extent of 0.4-1.2%.

The most suitable nitro-cellulose compound for carrying out this process contains 12.7-13% of nitrogen. It is however possible 100

satisfactorily to transform by the process into practice and sporting powder nearly all old powders, such as rifle and gun powder withdrawn from ordnance use or powder which, owing to low stability, must be destroyed.

5 The old powder or nitro-cellulose is incorporated with a mixture of alcohol and ether, acetone or other solvent in a quantity of 90-160% by weight of the dry mass with an addition of 0.1 to 0.5% of graphite and 4% to 10% of water as well as 0.4 to 1.2% of stabilizing substance. The mass is kneaded in a kneading apparatus for several hours and after extrusion the extruded threads are subjected to the hot fluid bath, as above described.

In the forcible evaporation of ether in the presence of oxygen and water or steam, peroxides are easily formed, which have a negative effect upon the stability of the powder. It is therefore advisable to add to the bath easily oxidized substances which have no such detrimental effect on the powder and which destroy the action of the peroxides (e. g. 0.1-1% of aniline, phenylurea, or nitrous or other reducing acids). When transforming old powders of reduced stability it is advisable to add 1-2% of substances which neutralize the acids (e. g. sodium hydrogen carbonate).

30 In view of the small thickness of the wall and the cylindrical, tubular, form of the thread, the ignition velocity of the powder is high, it being well known that this velocity is a function of the size of the grains.

What we claim is:

1. Method of manufacturing smokeless practice and sporting powder consisting in gelatinizing explosive material with gelatinizing solvents, extruding the gelatinized material in the form of cylindrical threads, superficially drying the extruded threads, plunging the threads in a fluid bath having a temperature above the boiling temperature of 40 at least one of the ingredients in the thread so that said ingredient evaporates and ejects the explosive material contained in the cylindrical-shaped hardened exterior leaving a tubular-shaped thread, partially drying the 45 tubular-shaped thread thus formed, cutting the partially dried threads so as to form thin-walled tubular grains, drying, soaking, polishing and coating, as set forth.

2. Method of manufacturing smokeless practice and sporting powder consisting in gelatinizing explosive material with alcohol and ether, extruding the gelatinized material in the form of thin threads, superficially drying the extruded threads, plunging the threads in a fluid bath having a temperature above the boiling temperature of at least one of the ingredients in the thread so that said ingredient evaporates and ejects the explosive material contained in the cylindrical-shaped 60 hardened exterior leaving a tubular-shaped

thread, partially drying the tubular-shaped thread thus formed, cutting the partially dried threads so as to form thin-walled tubular grains, drying, soaking, polishing and coating, as and for the purpose set forth.

3. Method of manufacturing smokeless practice and sporting powder consisting in gelatinizing explosive material with alcohol and ether, extruding the gelatinized material in the form of threads, superficially drying the extruded threads, plunging the threads in an aqueous fluid bath at 45-80° C. so that at least one of the ingredients evaporates and ejects the explosive material contained in the cylindrical-shaped hardened exterior leaving a tubular-shaped thread, partially drying the tubular-shaped thread thus formed, cutting the partially dried threads so as to form thin-walled tubular grains, drying, soaking, polishing and coating, as set forth.

4. Method of manufacturing smokeless practice and sporting powder consisting in gelatinizing explosive material with alcohol and ether, extruding the gelatinized material in the form of threads of 0.3-1.5 mm. diameter, superficially drying the threads by heating at 50° C. for 1-2 minutes, plunging the threads in an aqueous bath at 45-80° C. for 10-25 minutes so that at least one of the ingredients evaporates and ejects the explosive material contained in the cylindrical-shaped hardened exterior leaving a tubular-shaped thread, partially drying the tubular-shaped thread thus formed, cutting the partially dried threads so as to form thin-walled tubular grains, drying, soaking, polishing and coating, as set forth.

5. Method of manufacturing smokeless practice and sporting powder consisting in gelatinizing explosive material with alcohol and ether, extruding the gelatinized material in the form of threads, superficially drying the extruded threads, plunging the threads in an aqueous bath containing a reducing agent at 45-80° C. so that at least one of the ingredients evaporates and ejects the explosive material contained in the cylindrical-shaped hardened exterior leaving a tubular-shaped thread, partially drying the tubular-shaped thread thus formed, cutting the partially dried threads so as to form thin-walled tubular grains, drying, soaking, polishing and coating, as set forth.

6. Method of manufacturing smokeless practice and sporting powder consisting in gelatinizing explosive material with alcohol and ether, extruding the gelatinized material in the form of threads, superficially drying the extruded threads, plunging the threads in an aqueous fluid bath containing nitrous acid at 45-80° C., so that at least one of the ingredients evaporates and ejects the explosive material contained in the cylindrical-shaped hardened exterior leaving a tubular-shaped thread, partially drying the tubular-shaped

thread thus formed, cutting the partially dried threads so as to form thin-walled tubular grains, drying, soaking, polishing and coating, as set forth.

7. Method of manufacturing smokeless practice and sporting powder consisting in gelatinizing explosive material with gelatinizing solvents in presence of 0.1-5% of graphite, 6-10% of water and 0.4-1.2% of urea derivative, extruding the gelatinized material in the form of cylindrical threads, superficially drying the extruded threads, plunging the threads in a fluid bath having a temperature above the boiling temperature of one of the ingredients in the thread so that at least the said ingredient evaporates and ejects the explosive material contained in the cylindrical-shaped hardened exterior leaving a tubular-shaped thread, partially drying the tubular-shaped thread thus formed, cutting the partially dried threads so as to form thin-walled tubular grains, drying, soaking, polishing and coating, as set forth.

8. Method of manufacturing smokeless practice and sporting powder consisting in gelatinizing explosive material with gelatinizing solvents, extruding the gelatinized material in the form of cylindrical threads, superficially drying the extruded threads until they contain substantially equal amounts by weight of explosive material and the said gelatinizing solvents, plunging the threads in a fluid bath having a temperature above the boiling temperature of at least one of the ingredients in the thread so that said ingredient evaporates and ejects the explosive material contained in the cylindrical-shaped hardened exterior leaving a cylindrical-shaped thread, partially drying the tubular-shaped thread thus formed, cutting the partially dried threads, so as to form thin-walled tubular grains, drying, soaking, polishing and coating as set forth.

9. Method of manufacturing smokeless practice and sporting powder consisting in gelatinizing explosive material with alcohol and ether, extruding the gelatinized material in the form of threads, superficially drying the extruded threads until the weight of alcohol and ether contained therein is substantially equal to the weight of the said explosive material, plunging the threads in an aqueous fluid bath at 45-80° C. so that at least one of the ingredients evaporates and ejects the explosive material contained in the cylindrical-shaped hardened exterior leaving a tubular-shaped thread, partially drying the tubular-shaped thread thus formed, cutting the partially dried threads, drying, soaking, polishing and coating so as to form thin-walled tubular grains, as set forth.

10. Method of manufacturing smokeless practice and sporting powder consisting in gelatinizing explosive material with alcohol

and ether, extruding the gelatinized material in the form of threads, superficially drying the extruded threads until the weight of alcohol and ether therein is substantially equal to the weight of explosive material, plunging the threads in an aqueous bath containing a reducing agent at 45-80° C. so that at least one of the ingredients evaporates and ejects the explosive material contained in the tubular-shaped hardened exterior leaving a tubular-shaped thread, partially drying the tubular-shaped thread thus formed, cutting the partially dried threads so as to form thin-walled tubular grains, drying, soaking, polishing and coating, as set forth.

11. Method of manufacturing smokeless practice and sporting powder consisting in gelatinizing explosive material with alcohol and ether, extruding the gelatinized material in the form of threads of 0.8-1.5 mm. diameter, superficially drying the threads by heating at 50° C. until the weight of alcohol and ether contained therein is substantially equal to the weight of the said explosive material, plunging the threads in an aqueous bath at 45-80° C. for 10-25 minutes so that at least one of the ingredients evaporates and ejects the explosive material contained in the cylindrical-shaped hardened exterior leaving a cylindrical-shaped thread, partially drying the tubular-shaped thread thus formed, cutting the partially dried threads, so as to form thin-walled tubular grains, drying, soaking, polishing and coating, as set forth.

12. Method of manufacturing smokeless practice and sporting powder consisting in gelatinizing explosive material with alcohol and ether, extruding the gelatinized material in the form of threads, superficially drying the extruded threads until the weight of alcohol and ether therein is substantially equal to the weight of the explosive material, plunging the threads in an aqueous fluid bath containing nitrous acid at 45-80° C. so that at least one of the ingredients evaporates and ejects the explosive material contained in the cylindrical-shaped hardened exterior leaving a tubular-shaped thread, partially drying the tubular-shaped thread thus formed, cutting the partially dried threads so as to form thin-walled tubular grains, drying, soaking, polishing and coating, as set forth.

In testimony whereof we have signed our names to this specification.

EUGENIUSZ BAZYLEWICZ-KNIAZYKOWSKI.

KAZIMIERZ PARTYKA.

70

75

80

85

90

95

100

105

110

115

120

125

130